

# UNITED STATES PATENT OFFICE.

JAMES G. VAIL, OF CHESTER, AND JOHN D. CARTER, OF LANSDOWNE, PENNSYLVANIA.

## PROCESS OF FORMING AND BINDING MATERIAL FOR USE IN ABRASIVE WHEELS AND THE LIKE.

1,139,739.

Specification of Letters Patent. Patented May 18, 1915.

No Drawing.

Application filed November 4, 1913. Serial No. 799,105.

*To all whom it may concern:*

Be it known that we, JAMES G. VAIL and JOHN D. CARTER, citizens of the United States, and residents of Chester, county of Delaware, and State of Pennsylvania, and of Lansdowne, county of Delaware, and State of Pennsylvania, respectively, whose post-office addresses are the same, have invented a certain new and useful Process of 5 Forming and Binding Material for Use in Abrasive Wheels and the like, of which the following is a specification.

Various attempts have been made in the past to utilize alkaline solutions of the 15 various silicates, notably silicates of potassium and of sodium, as a binding material in forming abrasive wheels and similar articles, it having been found that wheels made with such binding materials are especially 20 adapted for certain classes of work. However, while it has been possible to produce a satisfactory wheel with a binding material of this nature when the abrasive material employed was emery, and possibly 25 certain other materials, it has hitherto been impossible to produce a commercially satisfactory article when carborundum is made use of as the abradant.

The principal objects of our invention are 30 to provide a process by which an abrasive wheel or similar article in which carborundum, or other substance having substantially similar chemical properties, is employed as the abradant, may be formed by the use of 35 solutions of alkaline silicates as a binding medium, and which when finished shall possess extreme hardness and durability, shall be efficient in operation, and in which the component particles of the abradant shall be 40 so firmly bound together that the tendency to burst when rotated at high speed shall be negligible; to provide such a process, which may be readily, cheaply and effectively carried out in factories at present engaged in 45 the manufacture of abrasive wheels, and with the machinery now in use; to provide a binding material for use in wheels and similar articles, and in furnace linings and the like in which carborundum, or other substance 50 having substantially similar chemical properties, is employed, which shall serve to firmly unite the particles together, and by the employment of which new and superior results will be obtained; and to provide an

abrasive wheel or the like of new and ad- 55 vantageous properties.

A further object of our invention is to provide a process of forming abrasive wheels in which carborundum or the like is employed as the abradant, which shall permit 60 of the use of webs within the wheels, should it be desired to employ them.

Our invention further includes all of the various other novel features and operations hereinafter more definitely specified. 65

In the manufacture of abrasive wheels and similar articles, as now carried on, in which the binding material consists of an alkaline solution of a silicate, it is customary to mix together the abradant material, 70 a hydrous clay or similar substance which may be termed the filler, and the binding material. The mixing of these substances may be performed in any convenient order, and in any desired proportions, a quantity 75 of the binding material, which may consist of a strongly alkaline solution of silicate of sodium or a somewhat similar silicate, being employed preferably sufficient to reduce the mixture to a plastic mass of the desired 80 consistency. This after being thoroughly mixed may be forced into suitable molds and baked at relatively moderate temperatures until the excess moisture is eliminated, 85 after which the finished wheel may be withdrawn from the mold. If it be desired to produce a wheel having a web, the metallic netting, or other material of which the web is formed, is introduced within the mold after a portion of the plastic substance has 90 been placed therein, the addition of the balance of the material serving to completely embed the web within the substance, after which the baking is carried out in the usual manner. 95

This process, although quite satisfactory where emery or certain other abradants are used, has not been found satisfactory for the production of wheels and similar articles in which carborundum is employed as the 100 abradant, as the wheels made thereby possess numerous disadvantages, among which may be mentioned their softness, inferior cutting quality, and tendency to disintegrate when in operation, thus practically 105 prohibiting their commercial use. It has, therefore, been customary to bind the particles of carborundum together by the use

of a ceramic bond, the material from which the bond is formed being placed in a suitable mold together with the carborundum and the filler, if the latter be employed, and the whole mass fused together at a high temperature. This method, while producing a wheel suitable for certain uses, does not produce a wheel having the advantages of one formed with a binder comprising a solution 10 of an alkaline silicate, and, moreover, the employment of webs within a wheel formed in this manner is impossible, as the heat necessary to properly fuse the ceramic material used as a binder, also serves to melt the 15 metallic web, thus rendering it useless.

We have found, however, that an alkaline solution of a suitable silicate may satisfactorily be employed as a binder for carborundum, or other substances having substantially similar chemical properties, by the 20 employment of a suitable oxidizing agent during the carrying out of the process of forming the wheel or like article, and that a wheel may thus be produced having none 25 of the disadvantages of the carborundum wheels employing ceramic binders, while possessing distinct advantages of its own. While it is possible to utilize various oxidizing agents with good results, we have 30 found that in practice a suitable amount of potassium permanganate, preferably in crystal form, although this is not essential, may be satisfactorily employed, and that excellent results may be obtained by the mixture 35 of, for example, say five per cent. by weight of this substance with an alkaline solution of sodium silicate in strength of, say, 60° Baumé, preferably while the latter is heated. While the addition of the oxidizing agent 40 may take place at any suitable time during the process of preparing the plastic mass out of which the wheel or other article is formed, the oxidizing agent may preferably be added to the silicate solution previous to 45 the addition of the latter to the carborundum and hydrous clay or other filling material. The proportions of the carborundum or like substance and hydrous clay, or other filling material, employed may be 50 regulated as may be desired, and after the addition of the binding material, composed of the silicate solution containing the potassium permanganate or other oxidizing agent, the resulting plastic mass may be treated in 55 a manner similar to that now employed in the manufacture of silicate wheels employing emery or other like substance as the abradant.

It seems probable that the difficulties previously encountered when efforts were made 60 to form an abrasive wheel in which carborundum, or other substance of substantially similar chemical properties, was employed as the abradant and an alkaline solution of a silicate as the binding material, arose from

the presence of free hydrogen gas liberated by the action of the alkaline silicate upon the carborundum, this gas probably forming either minute bubbles within the mass, or else enveloping the particles of carborundum 70 with a sort of sheath or coating, and preventing the binding material from properly adhering thereto. It is thought, however, that the oxygen in the oxidizing agent which we employ, by combining with the liberated 75 hydrogen to form water, practically eliminates the objectionable hydrogen gas, and thus permits the binding material to exert its maximum strength. It will thus be evident that the same result may be accomplished 80 whether a relatively concentrated solution of an alkaline silicate be employed, or whether a less concentrated solution, to which has been added caustic soda or caustic potash, or similar substances, be made use 85 of, as the oxidizing agent will, in any case, serve to combine with the gas which may be generated and which by its presence may serve to impede the action of the binding material.

Furthermore, it will be noted that our process may be employed with good results in any case where it be desired to firmly unite particles of material other than carborundum with a binder comprising a solution of an alkaline silicate, wherever the 95 nature of the particles be such that their contact with the binding material will serve to liberate uncombined gas within the mixture.

Furthermore, if desired, webs formed of practically any material may be employed in wheels formed according to our process, as the temperatures necessary to properly 100 bake the wheel are not sufficient to in any way affect the web, and it is possible, therefore, by the use of our process to produce a carborundum wheel having a web formed of material which melts at a comparatively low temperature.

In the carrying out of our process, we do not desire to limit ourselves to any fixed sequence of steps, as it will be evident that the oxidizing agent which is employed may be introduced with satisfactory results at 115 various points therein, although in practice we have found it desirable to combine the same with the binding material previous to its mixture with the carborundum, nor do we desire to limit ourselves to the employment of any specific oxidizing agent.

Furthermore, it will be evident that a suitable binding material for use in our process may be manufactured as a separate industry apart from the manufacture of 125 the wheels or other articles themselves, and may be utilized in the production of linings for furnaces and for many other purposes, as well as in the production of wheels and the like, and we desire to cover the manu- 130

facture of such substance, as well as the substance itself.

Finally, it will be evident that various changes may be made in our invention, as 5 herein described, and in the various steps of our process, as well as in the method of effectuating and carrying out the same, without departing from the spirit and scope of our invention as defined in the appended 10 claims.

Having thus fully described our invention, we claim and desire to protect by Letters Patent of the United States:

1. The process of forming an abrasive 15 wheel or the like, which comprises the use of carborundum, an alkaline solution of a silicate and an oxidizing agent soluble therein.

2. The process of forming an abrasive 20 wheel or the like, which comprises the use of an alkaline solution of sodium silicate, and potassium permanganate.

3. The process of forming an abrasive 25 wheel or the like which consists in combining an abradant capable of yielding hydrogen gas when in contact with an alkali with a binding material comprising an alkaline solution of a silicate and an oxidizing agent soluble therein, and then baking the resulting 30 mass in molds suitable to produce articles of the shape desired.

4. The process of forming an abrasive

wheel or the like, which consists in mixing carborundum with a suitable filler, reducing the mixture thus formed to a plastic 35 consistency by the addition of an alkaline solution of a silicate in combination with a suitable oxidizing agent, introducing the plastic mass into suitable molds, and baking the same at a relatively low temperature. 40

5. The process of forming an abrasive wheel or the like which consists in mixing carborundum with a suitable filler reducing the mixture to a suitable consistency by the addition of a binding material comprising 45 a solution of sodium silicate and potassium permanganate, introducing the resulting product into suitable molds and baking the same at relatively low temperatures.

6. As a new article of manufacture, a 50 molded abrasive wheel or the like formed of a composition comprising a suitable abradant yielding hydrogen gas when in contact with an alkali, a solution of an alkaline silicate, and an oxidizing agent soluble 55 therein.

In witness whereof we have hereunto set our hands this 3rd day of November, 1913.

JAMES G. VAIL.  
JOHN D. CARTER.

Witnesses:

ALEXANDER PARK,  
GEORGE K. HELBERT.